

Feb. 16, 1954

J. N. DALTON ET AL

2,669,002

PROCESS FOR SETTING WOOL FABRICS

Filed March 23, 1951



INVENTORS  
JOHN N. DALTON  
WILLIAM R. KAUPIM  
BY *S. J. Dalton*  
ATT'Y

## UNITED STATES PATENT OFFICE

2,669,002

## PROCESS FOR SETTING WOOL FABRICS

John N. Dalton, Providence, R. I., and William B. Kaupin, Lawrence, Mass., assignors to Pacific Mills, Lawrence, Mass., a corporation of Massachusetts

Application March 23, 1951, Serial No. 217,292

2 Claims. (Cl. 28—76)

1

This invention relates to a continuous process for the permanent setting of wool fabrics, by which we mean fabrics of all wool or of mixtures of wool, mohair, alpaca, etc., with nylon, regenerated cellulose, cellulose acetate, Vicara, Fiber V (now known as "Dacron"), Orlon, etc. By permanent setting we mean resistant to boiling water for at least 1 hour as in subsequent dyeing and to steaming as in pressing.

A principal object of the invention is to provide a continuous, rapid and inexpensive process for fixing in a permanent and regular manner the warp and filling threads by the removal of all irregular and hidden strains while the fabric is flat, thus preventing the formation of cockles, crimps, creases or other forms of uneven shrinkage at later stages of manufacture, such as mill scouring, dyeing, finishing, steaming and sponging. A further object is to prevent movement in the warp and filling directions in the finished cloth, which is shown by shrinkage, bubbling, or puckering when the fabric is exposed to steaming or to elevated humidity as in pressing or cleaning. A further object is to provide a process of this character which is readily controlled. A further object is to avoid the defects of the conventional batch processes.

The most common operation now in use for setting wool fabrics is "crabbing," with or without "blowing." Crabbing consists in winding the fabric under tension on a roller through boiling water. By this means the cloth is set but unless the work is carefully done many defects occur. The effectiveness of the process is governed by the tension at which the cloth is wound on the roller, the temperature and time of treatment, and the composition of the crabbing liquor. It is essential that each of these factors should be accurately controlled. The tension should be uniform but not too great or the handle of the fabric will be papery; the temperature of setting should be maintained constant; and the pH of the liquor should be maintained at about 7. Crabbing may be followed by blowing.

Blowing, which is used after crabbing, consists of forcing steam through the fabric, which is wrapped on a perforated roller. The cloth is held under tension warpwise, but is allowed to shrink in the filling direction; the cloth may shrink two or three inches in width, but the set remaining is relatively permanent. In both crabbing and blowing the process is a batch process and is slow and expensive and unless properly and carefully controlled the results are not wholly satisfactory. Blowing always lowers the tensile strength and

2

renders the fabric difficult to dye and subject to "listing." Then blown cloth dyes differently from unsteamed cloth and it is difficult or impossible to obtain uniform results. Our process gives a set as good as or better than crabbing and blowing, but without these defects and disadvantages and at lower cost.

In the accompanying drawing,

Fig. 1 is a schematic elevation partly in section of apparatus by means of which our process may be practiced, showing the part of the apparatus through which the cloth is first passed, and

Fig. 2 is a similar schematic elevation of the remainder of the apparatus.

According to our invention, the grey fabric, as it is continuously advanced in open width, is first impregnated with an aqueous solution of pH range 9 to 12. The impregnating solution may be a buffered solution such as sodium hydroxide and disodium phosphate, sodium hydroxide and boric acid, etc., or it may be a solution of an organic derivative of ammonia such as an amine.

In our preferred practice the open fabric 2, which has not previously been wet with water, is passed through a three-roll mangle having a tank 4 containing the impregnating solution so that the fabric is given two dips and two nips. The squeezed fabric retains more than 20%, and preferably about 50% to 60%, of its weight of the impregnating liquor after the final nip. The impregnated fabric is passed under a dancer roll 6 where the warp tension is adjusted and then fed onto a tenter at 8. The fabric on the tenter, adjusted with tension to the proper width, is so heated throughout its thickness that steam is generated in the interior of the fabric which coacts with the liquid in the fabric to set the yarns of the fabric.

To provide such heating we prefer to pass the fabric between banks of infra-red lamps 10, 12, over and under the traveling fabric.

For best results we use an upper bank 10 of 565 lamps and a lower bank 12 of 625 lamps, which banks are spaced 14 inches apart with the cloth in the middle. The banks are about 3 yards long on the tenter and are of sufficient width to cover the fabric, which generally is 5 feet wide. The fabric travels at a speed of 25 to 35 yards a minute and thus is maintained between the banks of lamps for from about 21 to 14 seconds. The lamps are 375 watts each, making a total of about 446 kilowatts, and providing over 25,000 B. t. u. per minute. Thus the cloth traveling at 25 yards per minute receives a heat input of over 67 B. t. u. per square foot and when

traveling at 35 yards per minute a heat input of over 48 B. t. u. per square foot. The number or size of the lamps may be varied to give a heat input between about 15,000 and 35,000 B. t. u. per minute.

The fabric passes out of the tenter while still damp and containing more than 20%, preferably 20% to 25%, of its weight of the impregnating liquor.

The fabric is then scoured in a continuous washer 14.

Our process has many advantages in the ease with which it may be controlled. The pH of the impregnating liquid is easy to regulate. The amount of pickup of such liquid can be readily controlled. The number of lamps in the banks in the tenter may be varied as well as the speed of the fabric through the tenter thereby controlling the generation of steam throughout the damp fabric. The dampness or moisture content of the fabric as it comes from the tenter may likewise be readily controlled. Both warp and weft tension may be independently controlled. In these particulars our process has great practical advantages over the batch processes for setting wool fabrics now in use.

We claim:

1. A continuous process for imparting to wool fabrics a permanent set resistant to mill scouring, dyeing, finishing, steaming and sponging which comprises continuously advancing the fabric in open width, wetting the traveling fabric by impregnating it with an aqueous solution of pH 9 to 12, subjecting the wet traveling fabric from both sides for about 14 to 21 seconds to high intensity infra-red radiation to generate steam in

the interior of the fabric, while maintaining said fabric under warpwise and weftwise tension, discontinuing application of infra-red radiation while the fabric contains more than 20% of its weight of the impregnating liquor, and thereafter scouring the fabric in a continuous washer.

2. A continuous process for imparting to wool fabrics a permanent set resistant to mill scouring, dyeing, finishing, steaming and sponging which comprises continuously advancing the fabric in open width, wetting the traveling fabric by impregnating it with an aqueous solution of pH 9 to 12, generating steam in the interior of the wet traveling fabric for about 14 to 21 seconds to coact with the liquid in the fabric to set the yarns of the fabric, while maintaining said fabric under warpwise and weftwise tension, discontinuing the generation of steam while the fabric contains more than 20% of the weight of the impregnating liquor, and thereafter scouring the fabric in a continuous washer.

JOHN N. DALTON.  
WILLIAM B. KAUPIN.

25 References Cited in the file of this patent

UNITED STATES PATENTS

| Number    | Name         | Date          |
|-----------|--------------|---------------|
| 2,132,156 | Gessner      | Oct. 4, 1938  |
| 2,251,127 | Gessner      | July 29, 1941 |
| 2,379,653 | Ridley       | July 3, 1945  |
| 2,499,444 | Allison      | Mar. 7, 1950  |
| 2,508,007 | Block et al. | May 16, 1950  |

FOREIGN PATENTS

| Number  | Country       | Date          |
|---------|---------------|---------------|
| 546,529 | Great Britain | July 17, 1942 |